

1

3,122,517

SPIN-DYEING OF ACRYLONITRILE POLYMERS  
 Winfried Kruckenberg, Leverkusen-Bayerwerk, and Adam Schultheiss, Dormagen, Germany, assignors to Farbenfabriken Bayer Aktiengesellschaft, Leverkusen, Germany, a corporation of Germany  
 No Drawing. Filed Oct. 17, 1958, Ser. No. 767,771  
 Claims priority, application Germany Oct. 18, 1957  
 6 Claims. (Cl. 260—41)

The present invention relates to the spin-dyeing of acrylonitrile polymers; more particularly it concerns a process wherein polyacrylonitrile or interpolymers of acrylonitrile and other copolymerisable compounds containing at least 70% acrylonitrile are spin-dyed by means of basic dyestuffs which are soluble in the solvents used for the spinning, for instance in dimethyl formamide, dimethyl sulfone, ethylene carbonate or nitro methane.

According to the present invention basic dyestuffs are used in the spin-dyeing of the acrylonitrile polymers which have been precipitated from their aqueous solutions.

These precipitated basic dyestuffs show a surprising increase of the solubility in the solutions serving for the spinning of the acrylonitrile polymers; with the aid of the precipitated basic dyestuffs, stock dyestuff solutions for example can be prepared for the spin dyeing which are made up with a significantly higher dyestuff content than hitherto possible. This applies particularly when dimethyl formamide is used as solvent. Moreover, the basic dyestuffs to be used according to the invention in the spinning process no longer give rise to troubles such as were frequently to be observed in the use of the water soluble basic starting dyestuffs on account of frequently entrained water soluble foreign salts. It is also noteworthy that the spinning masses treated with the proposed basic dyestuffs yield threads or fibres which possess a fastness to cross-dyeing which is better than that of threads or fibres obtainable from spinning masses which have been treated in the conventional manner with the corresponding water soluble dyestuffs. Contrary to most of the inorganic or organic pigments the basic dyestuffs which were precipitated from their aqueous solutions do not tend to clog the spinning nozzles; furthermore they do not bleed when the filaments are stretched in the precipitating bath.

To obtain the basic dyestuffs to be applied according to the invention one can for example proceed by dissolving the basic dyestuffs produced in a customary manner and which can belong to the most various series—e.g. the triphenyl methane series, the anthraquinone series, the azo series, the methine series or the phthalocyanine series—in water and then adding sulfonic acids or water soluble salts of sulfonic acids to the aqueous solutions. As suitable sulfonic acids, aliphatic acids and aromatic acids come into consideration such as, for example, propane-1,3-disulfonic acid, benzene mono- or disulfonic acid, naphthalene mono- or polysulfonic acid, diphenyl-4-sulfonic acid and condensation products of formaldehyde with naphthalene sulfonic acid or with 4,4'-dihydroxy diphenyl sulphone containing sulfonic acid groups. Instead of the sulfonic acids or their salts also other acids, such as maleic acid, fumaric acid, adipic acid, citric acid, trichloro acetic acid, borofluoro acetic acid, borofluoro butyric acid and hydrofluoboric acid or their water soluble salts may be used for precipitation. As water soluble salts the alkali metal salts are especially suitable.

The precipitation of the basic dyestuffs with the acids or their water soluble salts from the aqueous solutions can be effected in the cold or also with warming, the most suitable temperature being readily determinable in each case by preliminary experiments. The suitable proportions of the components can also be determined by pre-

2

liminary experiments without difficulty; in general it is recommended to apply the acids or their salts in a slight excess in relation to stoichiometric quantity.

The basic dyestuffs to be used according to the invention for spin dyeing acrylonitrile polymers include also those basic dyestuffs of the azo series which are precipitated by adding the acids or their salts which come into consideration already during the production of the azo dyestuffs, for instance during coupling, instead of after the production of the azo dyestuff.

The dyestuffs in the present case can, as is customary, be introduced into the spinning masses in the form of stock solutions; stock solutions made up with dimethyl formamide can contain for example 15-20% acrylonitrile polymer and 10-30% dyestuff.

#### Example 1

A 20% solution of polyacrylonitrile prepared in the usual manner in dimethyl formamide is treated with 0.5% of one of the basic dyestuffs described below, and then spun in a manner known as such. The dyeing of the fibres thus obtained is of outstanding fastness.

The dyestuffs used were obtained in the following manner: 75 g. of the red dyestuff of the formula



30 or of the formula



were dissolved in 750 ml. of water at 55° C. There was then added with good stirring within 15 minutes 150 g. of 40% aqueous solution of the sodium salt of the condensation product of formaldehyde with 4,4'-dihydroxy diphenyl sulfone containing sulfonic acid groups. The reaction mixture was further stirred for half an hour and then cooled to 20-25° C. The precipitated red dyestuff was filtered off with suction, washed with water and dried. For the precipitation of the dyestuffs 120 g. of a 25% aqueous solution of sodium propane-1,3-disulfonate or 40 ml. of borofluoro acetic acid or 40 ml. of hydrofluoboric acid ( $D_{20}^{\circ} 1.22$ ) can be used instead of 150 g. of the 40% aqueous solution of the condensation product.

#### Example 2

The procedure described in Example 1 is followed but instead of the basic dyestuffs used for the spin dyeing, a basic dyestuff is applied which has been precipitated by adding 190 ml. of the 40% solution of the condensation product of Example 1 at 55° C. to an aqueous solution of 90 g. of the yellow dyestuff of the formula



The dyestuff can also be used which precipitates if the above mentioned aqueous solution of the yellow dyestuff is treated, instead of with the 40% aqueous solution of the condensation product of Example 1, with a 40% aque-

ous solution of the condensation product of formaldehyde and sodium naphthalene sulfonate or sodium naphthalene 1,5-disulfonate.

*Example 3*

The procedure of Example 1 is followed, but instead of the dyestuffs used, the basic dyestuff is applied which precipitates if a solution of 20 g. of the orange coloured dyestuff of the formula



is treated at 55° C. with 50 ml. of the 40% aqueous solution of the condensation product applied in Example 1.

*Example 4*

The procedure described in Example 1 is followed but instead of the dyestuffs described the basic dyestuff is used which precipitates if at 55° C. the aqueous solution of 20 g. of the blue-black dyestuff of the formula



is treated with an aqueous solution of 15 g. of sodium naphthalene-1,5-disulfonate or 15 g. of sodium diphenyl-4-sulfonate.

*Example 5*

The procedure of Example 1 is followed but instead of the dyestuffs described, the basic dyestuff is used which precipitates if a solution of 60 g. of the violet dyestuff of the formula



is treated in 700 ml. of water at 80° C. as described in Example 1 with 75 ml. of the 40% aqueous solution of the condensation product indicated in Example 1.

*Example 6*

For the spin dyeing as described in Example 1 a basic dyestuff is used which has been obtained in the following way:

To 450 ml. of 30% hydrochloric acid, 100 g. of 2-amino-5-chloro-benzo-trifluoride are added dropwise with stirring in the course of 1½ to 2 hours. The mixture is then further stirred for several hours and then cooled by external cooling to a temperature below 0° C. A solution of 36 g. of sodium nitrite in 70 ml. of water is thereupon added dropwise within two hours, care being taken that the temperature does not rise above 0° C. After the reaction mixture has been stirred for a further 30 minutes it is filtered. The slight excess of nitrite in the filtrate is removed with amido sulfonic acid and the diazo solution is then poured into a solution prepared by dissolving 100 g. of naphthalene-1,5-disulfonic acid and 160 g. of N-ethyl-N-phenyl-β-amino-ethyl-trimethyl-ammonium chloride in 600 ml. of water. The mixture is partially neutralized, with further addition of ice, with concentrated caustic soda to a pH of 5.5 to 6.5 and stirred for another hour. The dyestuff which has meanwhile separated out is then filtered off with suction, washed free from salt with water and dried at 50–60° C.

*Example 7*

The procedure described in Example 1 is followed using a basic dyestuff obtained in the following way: 50 g. of the blue dyestuff of the formula



are dissolved in 300 ml. water with the addition of 10 ml. of glacial acetic acid at 60–70° C. and this solution is added to another solution of 35 g. of sodium-α-naphthalene sulfonate in 200 ml. of water and containing 250 g. of ice. The precipitated dyestuff is then filtered off and dried.

*Example 8*

The procedure described in Example 1 is followed but instead of the basic dyestuffs used for the spin dyeing, a basic dyestuff is applied which was precipitated by treating an aqueous solution of 36 g. of the dyestuff of the formula



with an aqueous solution of 33 g. of naphthalene-1,5-disulfonic acid sodium salt.

*Example 9*

The procedure described in Example 1 is followed but instead of the basic dyestuffs used for the spin dyeing, a basic dyestuff is applied which has been precipitated in the following manner:

40 g. of the dyestuff of the formula



are dissolved in 300 ml. of water and to the aqueous solution there is added a solution of 26 g. of sodium citrate in 80 ml. of water or a solution of 22.5 g. of sodium maleate in 20 ml. of water. After cooling the mixture to 20° C. the precipitated basic dyestuff is filtered off with suction, washed with water and dried at 50–60° in vacuo.

We claim:

1. In the process of spin-dyeing acrylonitrile polymers with basic dyestuffs which are soluble in the solvent used for the spinning, the step which comprises using basic dyestuffs which have been precipitated from their aqueous solution by means of a member selected from the group consisting of an aromatic sulfonic acid and a water soluble salt of an aromatic sulfonic acid, said member having at least 2 aromatic rings.

2. The process of claim 1 wherein the member is the sodium sulfonate of the condensation product of formaldehyde with 4,4'-dihydroxy diphenyl sulfone.

3. The process of claim 1 wherein the member is the condensation product of formaldehyde and sodium naphthalene sulfonate. 5

4. The process of claim 1 wherein the member is sodium naphthalene 1,5-disulfonate.

5. The process of claim 1 wherein the member is sodium diphenyl-4-sulfonate.

6. The process of claim 1 wherein the member is 10 sodium- $\alpha$ -naphthalene sulfonate.

References Cited in the file of this patent

UNITED STATES PATENTS

|           |                   |                |
|-----------|-------------------|----------------|
| 2,811,515 | Stocker           | Oct. 29, 1957  |
| 2,875,211 | Seibert et al.    | Feb. 24, 1959  |
| 2,906,588 | Brunkhorst et al. | Sept. 29, 1959 |
| 2,941,970 | Craig             | June 21, 1960  |

FOREIGN PATENTS

|         |               |               |
|---------|---------------|---------------|
| 616,440 | Great Britain | Jan. 21, 1949 |
| 686,269 | Great Britain | Jan. 21, 1953 |

OTHER REFERENCES

Fierz-David and Blangey: Fundamental Processes of Dye Chemistry, Interscience Pub. Inc., New York, 1949.